

June 22, 1937.

N. P. GOSS

2,084,337

METHOD OF ROLLING MAGNETIC MATERIAL

Filed Dec. 1, 1934

*Fig. 1.*



*Fig. 2.*



STRIP COLD ROLLED  
TO FINISHED GAUGE

*Fig. 3.*



INVENTOR

Norman P. Goss  
by his attorneys

Byrnes, Stabbins & Blenko

## UNITED STATES PATENT OFFICE

2,084,337

## METHOD OF ROLLING MAGNETIC MATERIAL

Norman P. Goss, Youngstown, Ohio, assignor, by  
mesne assignments, to Allegheny Steel Com-  
pany, Pittsburgh, Pa., a corporation of Penn-  
sylvania

Application December 1, 1934, Serial No. 755,575

3 Claims. (Cl. 80—60)

My invention relates to the making of magnetic material and, in particular, to the manufacture of such material in the form of thin sheets or laminations adapted for the assembly 5 of cores of electrical apparatus of various types.

This application is in part a continuation of my copending application Serial No. 718,789, filed April 3, 1934, for Metal rolling.

So-called "electrical sheets" have generally 10 been made heretofore by hand on a two-high hot mill. In my Patent No. 1,965,559, I have disclosed a method of producing a highly superior grade of magnetic material by cold rolling and heat treating hot rolled strip. I have discovered 15 that the quality and characteristics of the final product, particularly its permeability at high flux densities, and hysteresis and eddy current losses, are determined not only by the procedure followed in reducing the hot strip to final gauge, but also by the processing of the slabs from 20 which the hot strip is rolled and, furthermore, the manufacture of the slabs from the ingots. While the invention has particular reference to silicon steel containing about 3% or less of 25 silicon, it is not limited thereto and may be utilized in the manufacture of any magnetic material, regardless of composition.

For a complete understanding of the invention, reference is made to the accompanying drawing illustrating the invention diagrammatically and the appended description relating thereto. In the drawing:

Figure 1 is a diagram illustrating the manufacture of slabs from the ingot;

Figure 2 is a diagram illustrating the manufacture of strip from the slabs; and

Figure 3 is a diagram illustrating the manufacture of the finished product from the hot strip.

In accordance with my invention, I prepare a melt of silicon steel containing 3% silicon or less, and pour it into ingots of any convenient size. After solidification, the ingots are heated to a temperature of about 2000° F. or above.

They are then ready to be rolled into slabs. This stage of the operations is shown diagrammatically in Figure 1 of the drawing.

The ingot 10 may be reduced to slab form by any convenient means, rolling, forging, or otherwise, but I preferably subject the ingot to rolling in a suitable rolling mill 11 and shear the resulting product into slabs 12. I preferably complete the rolling of the ingot into slabs at one heat, the slabs being finished while at a temperature 55 of 1900° F. or below, determined by the natural

cooling of the ingot as it is rolled down into slab form.

The slabs 12 thus produced are reheated to a temperature of about 2000° F. or above. They are then ready for reduction to strip form, shown 5 at 13, which may best be accomplished by rolling, either in a continuous mill 14 or in a reversing mill, both of which are well known. For convenience, the material is preferably coiled during the later stages of the reduction into strip and, in any case, after the final reduction. This stage of the operations is indicated diagrammatically in Figure 2.

The rolling of the slab into strip form seems to exercise an effect upon the final results obtained as great as that of the rolling of the ingots. I have found that the greatly improved results are produced by heating the slab to a temperature of between about 2000° and 2100° F. for a period of time sufficient to permit thorough penetration of the heat into all parts of the slab uniformly, the time depending somewhat on the silicon content, and the nature of the practice followed in casting and finishing the ingot. For a 3% silicon steel, I prefer to heat the slabs to a temperature between about 2000° and 2050° and hold them at that temperature until the slab is thoroughly heated throughout, to the same temperature in all parts.

After heating to a temperature in the vicinity of 2000°—2100° F. for the time specified, which heating may be conducted in a convenient manner in any desired type of furnace, I remove the slabs from the heating zone and permit them to cool to a temperature such that when they have been rolled to final gauge, the temperature has decreased to a value sufficiently below the temperature of the first heat treatment to which the finished strip is subjected (usually about 1600° F.) to insure quick response to recrystallization on such subsequent heating. I prefer to finish the hot strip at 1450° F. or below, although good results may be obtained even if the strip is finished at a temperature as high as 1500° F. or 1550° F. Usually, it is highly desirable to permit the slabs to cool from their initial temperature to about 1900° before the rolling is started. In the ordinary continuous mill, the temperature will have been reduced from that figure to about 1450° by the time the rolling has been completed. It is possible to finish at a lower temperature, say 1200° or 1300° F. with equally satisfactory results, the prime consideration being to finish at a temperature not much higher than 1450°. This finish-

5

10

15

20

25

30

35

40

45

50

55

ing temperature seems to produce the best results.

The heating of the slabs initially to a temperature of about 2050° F. appears to be highly important. It has been found that if the slabs are initially heated to a higher temperature, say 2300° or 2200° F. and then finished, the results are not so good as when the slabs are heated only to 2050°, even though the strip is finished at 1450° F. or below.

Likewise, heating the slabs initially to about 1800°-1900° or less and rolling so that the strip is finished at 1450° or below, produces results which are not so good as those of the preferred method. The results obtained with a variety of practices differing slightly from the preferred method indicate the desirability of the latter as compared to any variant thereof.

The importance of finishing the strip at 1450° F. or below is demonstrated by the fact that in one mill, where it was necessary to roll the slab immediately on leaving the furnace due to the set-up of the mill, the strip was finished between 1550° and 1600° but the product was very inferior magnetically to that produced by the preferred method.

The initial heating of the ingot to a temperature of 2000° F., or above, is also of great importance. If the ingot is heated to only 1800° F., for example, and the resulting billets processed in accordance with the preferred practice outlined herein, the final product will not have characteristics as desirable as if the ingots were initially heated to 2000° or above before being formed into slabs.

After the hot strip has been rolled, coiled and cooled, it is ready for reduction in the cold to final gauge, in accordance with the disclosure of my above mentioned Patent No. 1,965,559. This stage of the operation is indicated diagrammatically in Figure 3, showing a four-high reversing mill 15 with winding and unwinding reels 16.

To generalize from the results of much experiment, I may say that, in addition to the method for reducing the hot strip in the cold to final gauge, disclosed in my patent aforementioned, the development of the most desirable quality in the final product appears to require the initial heating of both the ingot and slabs to a relatively high temperature, say 2000° F. or above, before reducing them respectively to slabs and strip, and the finishing of the hot rolled strip at a relatively much lower temperature, in the neighborhood of 1450° F.

I am aware that it has been proposed hereto-

fore to heat silicon steel containing upwards of 5% silicon, to a temperature of approximately 2000° for the purpose of increasing the ductility of the material. I do not believe that it has ever been proposed heretofore to improve the magnetic qualities of magnetic material by heating it to such temperatures in the ingot form, before reducing it to slabs and strip for the manufacture of thin magnetic sheets. I am also aware that it has been previously suggested to finish the hot rolling of silicon steel strip at a temperature of around 1400° F. It has not, however, been possible by such methods to obtain the desirable results flowing from my method, including the initial heating of the slab to a relatively high temperature, as well as the finishing of the hot rolling of the strip at a relatively much lower temperature.

While I have described herein but one preferred practice of the method of my invention, it will be apparent that certain changes therein may be made without departing from the spirit of the invention or scope of the appended claims.

For example, instead of subjecting the slab to a special cooling operation to insure that the strip will be finished at a temperature of 1450° F. or below, I may control the rate of rolling or the rate of cooling while rolling so as to produce the desired temperature in finishing, without any special intermediate cooling step.

I claim:

1. In a method of making magnetic material having improved magnetic properties, the steps including heating an ingot of silicon-iron alloy containing about 3% silicon to a temperature above 2000° F., reducing the ingot to slab form without reheating it, and reducing the slab to strip after heating the slab to about 2000° F., finishing at 1450° F. or below.

2. A method of making magnetic material the steps including heating an ingot of silicon steel containing about 3% silicon to a temperature of about 2000° F., reducing the ingot to slabs, heating the slabs to about 2000° F., reducing the slabs to strip and finishing the strip rolling while the material is at a temperature of about 1400° F.

3. In a method of making magnetic material having improved properties, the steps including heating an ingot of silicon-iron alloy containing about 3% silicon to a temperature above 2000° F. and rolling the ingot into strip, finishing the rolling of the strip when it is at a temperature of 1450° F. or below.

NORMAN P. GOSS. 55